

## [54] BINDER FOR CUTTING PARTICLES OF ABRASIVE TOOL

[76] Inventors: **Valentin Nikolaevich Bakul**, Kirova ul., 34-a, kv. 12; **Esfir Salimanovna Rabinovich**, Krasnopol'skaya ul., 20/15, kv. 25; **Jury Alexandrovich Yakovchuk**, Lesi Ukrainski bulvar, 3, kv. 42, all of Kiev, U.S.S.R.

[22] Filed: July 5, 1972

[21] Appl. No.: 269,136

## Related U.S. Application Data

[63] Continuation-in-part of Ser. No. 70,589, Sept. 8, 1970, abandoned.

[52] U.S. Cl. .... 260/19 U, 260/45.95 R, 260/826, 260/846, 260/847

[51] Int. Cl. .... C08g 5/20

[58] Field of Search .... 260/846, 826, 194, 845, 260/847, 45.95 R

## [56] References Cited

## UNITED STATES PATENTS

|           |         |             |           |
|-----------|---------|-------------|-----------|
| 2,659,708 | 11/1953 | Berger..... | 260/19 UA |
| 3,277,209 | 10/1966 | Giller..... | 266/19 U  |

## FOREIGN PATENTS OR APPLICATIONS

|         |         |                     |          |
|---------|---------|---------------------|----------|
| 514,858 | 7/1955  | Canada .....        | 260/19 U |
| 613,073 | 11/1948 | Great Britain ..... | 266/19 U |

Primary Examiner—Donald E. Czaja

Assistant Examiner—William E. Parker

Attorney, Agent, or Firm—Holman and Stern

## [57] ABSTRACT

A binder for cutting particles of an abrasive tool comprising a high-molecular component including butadiene-nitrile rubber in the amount of 100 parts by weight in combination with phenolformaldehyde resin in the amount of 10-30 parts by weight and with polyvinylchloride resin in the amount of 5-70 parts by weight, while the materials used for vulcanization, solidification, plasticization and stabilization of the ingredients of the high-molecular component include the following components taken in parts by weight

|                                         |          |
|-----------------------------------------|----------|
| sulphur                                 | 1.5-40.0 |
| zinc oxide                              | 3.0-20.0 |
| hexamethylenamine                       | 0.5-1.5  |
| plasticizers of polyvinylchloride resin | 5.0-40.0 |
| stabilizers of polyvinylchloride resin  | 0.5-3.0. |

5 Claims, No Drawings

**BINDER FOR CUTTING PARTICLES OF  
ABRASIVE TOOL**

This application is a continuation-in-part of application Ser. No. 70,589, filed Sept. 8, 1970, now abandoned.

The present invention relates to the field of manufacture of abrasive tools and, more particularly, the invention relates to binders for cutting particles of an abrasive tool.

The present invention can be most successfully used for making diamond polishing bands designed, for example, for treating journals of crankshafts of automobile and tractor engines.

Well known in the art are binders for cutting particles of an abrasive tool including a high-molecular component and materials used for vulcanization, hardening, plasticization and stabilization of the ingredients of the high-molecular component.

In the known binders for cutting particles of an abrasive tool the high-molecular component is a combination of butadiene-nitrile rubber with phenol-formaldehyde resin, while the materials used for vulcanization and solidification of these ingredients of the high-molecular component consist of sulphur, zinc oxide, magnesium oxide, 2,2-dithio-bis-benzothiazole, 2-mercaptopbenzothiazole, tetramethylthiuram disulphide, hexamethylenamine.

These binders provide for strong anchoring of the cutting abrasive particles, however, the binders themselves and the abrasive layers on the base thereof have a low plasticity and, therefore, are disadvantageous from the technological point of view: they are poorly rolled, calendered and shaped in the process of pressing. In this case, the addition of a plasticizing agent into the high-molecular component to avoid the above-mentioned disadvantages presents considerable technological difficulties.

The above disadvantages do not permit the binder to have a necessary elasticity and flexibility. Furthermore, the abrasive-containing layer made on the base of the known binders of the above-said types exhibits a poor wear resistance and is worn out before the high cutting properties of the abrasive tool, e.g., diamond, are completely utilized.

In the other known binders for cutting particles of an abrasive tool the high-molecular component is a combination of butadiene-nitrile rubber with a polyvinylchloride resin, whereas the materials used for vulcanization, plasticization and stabilization of the said ingredients of the high-molecular component consist of sulphur, zinc oxide, magnesium oxide, 2,2-dithio-bis-benzothiazole, 2-mercaptopbenzothiazole, tetramethylthiuram disulphide, dibutylphthalate, calcium stearate.

In these known binders the high-molecular component is easily mixed with plasticizers and, as a result, these binders feature good technological properties. However, these binders have a short life in operation, because they hold the cutting particles poorly due to their low adhesiveness.

An object of the invention is to eliminate the above-mentioned disadvantages.

The basic object of the invention is to develop a binder for cutting particles of an abrasive tool comprising such a high-molecular component which would provide for strong fixing of the cutting particles, would

have a high wear resistance and would be practical to make.

This object is attained by providing such a binder for cutting particles of an abrasive tool in which, according to the invention, the high-molecular component consists of butadiene-nitrile rubber in the amount of 100 parts by weight in combination with novolak phenol-formaldehyde resin in the amount of 10-30 parts by weight and polyvinylchloride resin in the amount of 5-70 parts by weight, whereas the materials used for vulcanization, solidification, plasticization and stabilization of the ingredients of the high-molecular component consist of the following ingredients (in parts by weight):

|    |                                         |             |
|----|-----------------------------------------|-------------|
| 15 | sulphur                                 | 1.5 to 40.0 |
|    | zinc oxide                              | 3.0 to 20.0 |
|    | hexamethylenamine                       | 0.5 to 1.5  |
| 20 | plasticizers of polyvinylchloride resin | 5.0 to 40.0 |
|    | stabilizers of polyvinylchloride resin  | 0.5 to 3.0  |

It is expedient to use dibutylphthalate as a plasticizer of polyvinylchloride resin and calcium stearate as a stabilizer of this resin.

The most advantageous solution of the problem is achieved in the case when the proposed binder for cutting particles besides the ingredients given hereinbelow in parts by weight:

|    |                                   |           |
|----|-----------------------------------|-----------|
| 30 | butadiene-nitrile rubber          | 100.0     |
|    | novolak phenol-formaldehyde resin | 10.0-20.0 |
|    | polyvinylchloride resin           | 40.0-60.0 |
| 35 | sulphur                           | 1.5-2.0   |
|    | zinc oxide                        | 3.0-5.0   |
|    | hexamethylenamine                 | 0.5-1.0   |
|    | dibutylphthalate                  | 25.0-35.0 |
|    | calcium stearate                  | 0.5-1.0   |

comprises the following compounds

|    |                               |         |
|----|-------------------------------|---------|
| 40 | 2-mercaptopbenzothiazole      | 1.5-2.0 |
|    | tetramethylthiuram disulphide | 0.5-0.8 |

It is also advantageous that proposed binder for cutting particles of an abrasive tool, besides the ingredients given in the following parts by weight:

|    |                                   |           |
|----|-----------------------------------|-----------|
| 50 | butadiene-nitrile rubber          | 100.0     |
|    | novolak phenol-formaldehyde resin | 10.0-20.0 |
|    | polyvinylchloride resin           | 40.0-60.0 |
|    | sulphur                           | 20.0-30.0 |
|    | zinc oxide                        | 10.0-20.0 |
|    | hexamethylenamine                 | 0.5-1.0   |
|    | dibutylphthalate                  | 25.0-35.0 |
|    | calcium stearate                  | 0.5-1.0   |

also comprises

|    |                              |          |
|----|------------------------------|----------|
| 60 | magnesium oxide              | 8.0-13.0 |
|    | 2,2-dithio-bis-benzothiazole | 1.8-2.3  |

It is preferable to use such a binder for cutting particles of an abrasive tool which, in addition to the ingredients given hereinbelow in parts by weight, i.e.:

|    |                                   |           |
|----|-----------------------------------|-----------|
| 65 | butadiene-nitrile rubber          | 100.0     |
|    | novolak phenol-formaldehyde resin | 20.0-25.0 |
|    | polyvinylchloride resin           | 5.0-10.0  |

## -Continued

|                   |           |
|-------------------|-----------|
| sulphur           | 35.0-40.0 |
| zinc oxide        | 10.0-20.0 |
| hexamethylenamine | 1.0-1.3   |
| dibutylphthalate  | 5.0-10.0  |
| calcium stearate  | 0.5-1.0   |

also comprises

|                               |          |
|-------------------------------|----------|
| magnesium oxide               | 8.0-13.0 |
| stearic acid                  | 1.0-1.5  |
| cumarone resin                | 5.0-10.0 |
| 2,2-dithio-bis-benzothiazole  | 1.8-2.3  |
| tetramethylthiuram disulphide | 0.5-0.7  |

Due to the above-mentioned compounds the proposed binder for cutting particles of an abrasive tool provides for strong anchoring of the cutting particles, has a high wear resistance and ensures wide technological facilities which make it possible to use this binder for making an abrasive tool with a variety of properties: from a soft, elastic and flexible tool to a hard and rigid one.

The invention is further described by way of example with a proposed table of compounds of the binders for cutting particles of an abrasive tool.

In the proposed binder for cutting particles of an abrasive tool the high-molecular component, according to the invention, consists of butadiene-nitrile rubber in the amount of 100 parts by weight in combination with novolak phenol-formaldehyde resin in the amount of 5-70 parts by weight, while the materials used for vulcanization, solidification, plasticization and stabilization of the ingredients of the high-molecular component and included into the compound of the binder comprise the following ingredients taken in parts by weight

|                                         |          |
|-----------------------------------------|----------|
| sulphur                                 | 1.5-40.0 |
| zinc oxide                              | 3.0-20.0 |
| hexamethylenamine                       | 0.5-1.5  |
| plasticizer of polyvinyl-chloride resin | 5.0-40.0 |
| stabilizers of polyvinyl-chloride resin | 0.5-3.0  |

To accelerate the process of vulcanization it is expedient to introduce additions of activators of the accelerators of vulcanization - zinc oxide and magnesium ox-

ide, additions of the accelerators - 2-mercaptopbenzothiazole and tetramethylthiuram disulphide, while in order to facilitate the process of mixing all components of the binder on rolls and for better dispersion of the cutting particles within the binder in the process of milling, besides the dibutylphthalate, coumarone resin and stearic acid are added.

In the process of mixing of the components of the binder on the rolls and during the vulcanization of the binder mixed with the cutting particles, the rubber interacts with the novolak phenol-formaldehyde resin. The polyvinylchloride resin accelerates this process. Simultaneous application of the rubber, novolak phenol-formaldehyde resin and polyvinylchloride resin in the binder in the above-said ratios makes it possible to obtain binders having a high wear resistance, capable of strongly retaining the cutting particles and being technologically convenient during the operations of milling, calendering, and shaping in the process of vulcanization.

By varying the amount of novolak phenol-formaldehyde and polyvinylchloride resin and other components relative to the amount of rubber, it is possible to obtain the binders having different properties: from soft and elastic to hard and rigid. Any increase of the content of novolak phenol-formaldehyde resin, sulphur and zinc oxide in the binder results in an increase of the rigidity of the binder. On the other hand, any increase of the amount of polyvinylchloride resin in conjunction with its plasticizer at a low content of sulphur and zinc oxide contributes to production of soft, elastic and wear-resistant binders.

The plasticizer of the polyvinylchloride resin consists of dibutylphthalate while the stabilizer of the same consists of calcium stearate.

Due to a wide range of the properties of the binder, the abrasive tool whose cutting particles are fixed in these binders features wide technological facilities.

An abrasive tool made on the soft elastic binders in the process of polishing provides for a high smoothness of the treated surface ( $R_a = 0.02-0.006$  microns) at a negligible removal of the material (in the order of 2-3 microns). The tool made on the rigid binders provides for smoothness of the treated surface up to  $R_a = 0.63-0.20$  microns at an increased removal of the material (in the order of 7-10 microns).

TABLE

of compounds of binders for cutting particles of abrasive tool

| Components                                                                                                                             | No.1  | Parts by weight |       |       |
|----------------------------------------------------------------------------------------------------------------------------------------|-------|-----------------|-------|-------|
|                                                                                                                                        |       | No.2            | No.3  | No.4  |
| <b>High-molecular component</b>                                                                                                        |       |                 |       |       |
| 1. Butadiene-nitrile rubber                                                                                                            | 100.0 | 100.0           | 100.0 | 100.0 |
| 2. Novolak phenol-formaldehyde resin                                                                                                   | 15.0  | 15.0            | 15.0  | 25.0  |
| 3. Polyvinylchloride resin                                                                                                             | 50.0  | 50.0            | 50.0  | 5.0   |
| Ingredients used for vulcanization, solidification, plasticization and stabilization of the components of the high-molecular component |       |                 |       |       |
| 4. Sulphur                                                                                                                             | 1.5   | 20.0            | 30.0  | 40.0  |
| 5. Tetramethylthiuram disulphide                                                                                                       | 0.5   | —               | —     | 0.6   |
| 6. 2-mercaptopbenzothiazole                                                                                                            | 1.5   | —               | —     | —     |
| 7. 2,2-dithio-bis-benzothiazole                                                                                                        | —     | 2.0             | 2.0   | 2.0   |

TABLE - Continued

| Components            | of compounds of binders for cutting particles of abrasive tool |                 |        |        |
|-----------------------|----------------------------------------------------------------|-----------------|--------|--------|
|                       | No.1                                                           | Parts by weight | No.3   | No.4   |
|                       | No.2                                                           |                 |        |        |
| 8. Zinc oxide         | 4.0                                                            | 15.0            | 15.0   | 15.0   |
| 9. Magnesium oxide    | —                                                              | 10.0            | 10.0   | 10.0   |
| 10. Hexamethylenamine | 0.75                                                           | 0.75            | 0.75   | 1.25   |
| 11. Dibutylphthalate  | 30.0                                                           | 30.0            | 30.0   | 5.0    |
| 12. Stearic acid      | —                                                              | —               | —      | 1.0    |
| 13. Coumarone resin   | —                                                              | —               | —      | 5.0    |
| 14. Calcium sterate   | 0.5                                                            | 0.5             | 0.5    | 0.5    |
| Total:                | 203.75                                                         | 243.25          | 253.25 | 210.35 |

## EXAMPLE 1

The compound of binder No. 1 given in the Table is recommended for making the soft high-elasticity binders used as a binding agent for cutting particles of an abrasive tool intended for polishing materials to a high degree of smoothness of the treated surface ( $R_a = 0.02\text{--}0.006$  microns).

Such a binder is used, for example, in manufacture of diamond elastic polishing disks designed for making metallographic and mineralographic microsections.

## EXAMPLE 2

Binder compound No. 2 given in the table is recommended for the elastic binders of an increased hardness used in preparation of a cutting layer of an abrasive tool employed when polishing materials to the surface smoothness corresponding to  $R_a = 0.08\text{--}0.025$  microns but at somewhat higher removal of the treated material (3-4 microns).

This binder is used, for example, in manufacture of diamond emery cloth designed for polishing semi-precious stones.

## EXAMPLE 3

Binder compound No. 3 given in the Table is recommended for preparing semi-rigid binders of the semi-ebonite used in making a cutting layer of an abrasive tool designed for polishing materials to the surface smoothness corresponding to  $R_a = 0.32\text{--}0.10$  micron, but at removal of the treated material up to 5-6 microns.

Such a binder is used, for example, in making diamond polishing bands employed for polishing steel and iron journal of crankshafts of automobile and tractor engines.

## EXAMPLE 4

Binder compound No. 4 given in the Table is recommended for preparing the rigid binders of the ebonite type used in making a cutting layer of an abrasive tool designed for treating materials to the surface smoothness corresponding to  $R_a = 0.63\text{--}0.20$  micron while removing the treated material for 7-10 microns.

Such a binder is used, for example, in making diamond bands employed for treating various steel members.

The above-said binders can be used for an abrasive tool applied on a carrier, e.g., a fabric in the form of a band, emery cloth, disks, or without any carrier base, i.e., grinding-and-polishing wheels, bars for finish honing, etc.

On making the bands, emery cloth, disks, the abrasive-containing layer consisting of the binder with dispersed cutting particles is anchored on a carrier by means of hot pressing and vulcanization in a usual way.

The wheels, honing bars and similar tools are usually made by means of hot moulding and vulcanization of the abrasive-containing layer in press-moulds.

The tool made with an abrasive-containing layer on the binders according to the invention provides for a high quality of the treatment and is characterized by high operational properties.

Thus, the use of the elastic diamond disks based on compound No. 1 (see the Table), as a binder makes it possible to obtain such a high quality of the surface of some materials like palladium, bimetal materials and various alloys, which was unachievable earlier through the use of the known tools. These disks are characterized by extremely high resistance and by stability of their properties. A set consisting of three disks of 200 mm in diameter comprising diamonds of various granularity can be used for making 3,000 to 6,000 high-quality metallographic microsections of steels and hard alloys of various grades; each having an area of 1.5 to 2.0  $\text{cm}^2$ . The resistance of the disks made on the base of this binder exceeds the resistance of the same disks made on the base of conventional binder at least by a factor of 1,000.

The experiments have shown that when using the compound of binder No. 3, according to the present invention, it is possible to make diamond bands having high resistance and stability and intended for treating steel members. For example, a single band with the dimensions of a diamond-containing layer of  $55.0 \times 43.5 \times 0.8$  is suitable for polishing 40,000 to 80,000 journals of steel crankshafts of automobile engines against 500 journals in the case of using the conventional bands of the same size made on the base of the known binders.

The high resistance of the tool and stability of its properties make it possible to mechanize and automate the processes of grinding and polishing effected with the aid of such a tool. In addition, it is possible to modernize the grinding-and-polishing equipment by eliminating the units intended, for example, for reeling and unreeeling the band and for automatically transferring the band after the treatment of each member.

Thus, the binders according to the present invention, make it possible to produce an abrasive layer having a high wear resistance, high capacity for holding cutting abrasive particles and good technological properties;

therefore, such a layer is featured by high operational characteristics.

What we claim is:

1. A binder for cutting particles of an abrasive tool comprising a high molecular component, said high molecular component consisting of 100 parts by weight of butadiene-nitrile rubber, 10 to 30 parts by weight of a novolak phenol-formaldehyde resin and 5 to 70 parts by weight of polyvinylchloride resin, and materials for vulcanization, solidification, plasticization and stabilization of said high molecular component, said materials comprising:

|                                        |          |
|----------------------------------------|----------|
| sulphur                                | 1.5-40.0 |
| zinc oxide                             | 3.0-20.0 |
| hexamethylenamine                      | 0.5-1.5  |
| plasticizer of polyvinylchloride resin | 5.0-40.0 |
| stabilizers of polyvinylchloride resin | 0.5-3.0  |

2. A binder as claimed in claim 1 in which the plasticizer of the polyvinylchloride resin consists of dibutylphthalate while the stabilizer thereof consists of calcium stearate.

3. A binder as claimed in claim 1 wherein said high molecular component and said materials are present in the following proportions, taken in parts by weight:

|                                   |           |
|-----------------------------------|-----------|
| butadiene-nitrile rubber          | 100.0     |
| novolak phenol-formaldehyde resin | 10.0-20.0 |
| polyvinylchloride resin           | 40.0-60.0 |
| sulphur                           | 1.5-2.0   |
| zinc oxide                        | 3.0-5.0   |
| hexamethylenamine                 | 0.5-1.0   |
| dibutylphthalate                  | 25.0-35.0 |
| Calcium stearate                  | 0.5-1.0   |

said binder further comprising:

|                               |         |
|-------------------------------|---------|
| 2-mercaptopbenzothiazole      | 1.5-2.0 |
| tetramethylthiuram disulphide | 0.5-0.8 |

5 4. A binder as claimed in claim 1 wherein said high molecular component and said materials are present in the following proportions in parts by weight:

|                                   |           |
|-----------------------------------|-----------|
| butadiene-nitrile rubber          | 100.0     |
| novolak phenol-formaldehyde resin | 10.0-20.0 |
| polyvinylchloride resin           | 40.0-60.0 |
| sulphur                           | 20.0-30.0 |
| zinc oxide                        | 10.0-20.0 |
| hexamethylenamine                 | 0.5-1.0   |
| dibutylphthalate                  | 25.0-35.0 |
| calcium stearate                  | 0.5-1.0   |

15 said binder further comprising:

|                              |          |
|------------------------------|----------|
| magnesium oxide              | 8.0-13.0 |
| 2,2-dithio-bis-benzothiazole | 1.8-2.3  |

20 5. A binder as claimed in claim 1 wherein said high molecular component and said materials are present in the following proportions in parts by weight:

|                                   |           |
|-----------------------------------|-----------|
| butadiene-nitrile rubber          | 100.0     |
| novolak phenol-formaldehyde resin | 20.0-25.0 |
| polyvinylchloride resin           | 5.0-10.0  |
| sulphur                           | 35.0-40.0 |
| zinc oxide                        | 10.0-20.0 |
| hexamethylenamine                 | 1.0-1.3   |
| dibutylphthalate                  | 5.0-10.0  |
| calcium stearate                  | 0.5-1.0   |

said binder further comprising:

|                               |          |
|-------------------------------|----------|
| magnesium oxide               | 8.0-13.0 |
| stearic acid                  | 1.0-1.5  |
| coumarone resin               | 5.0-10.0 |
| 2,2-dithio-bis-benzothiazole  | 1.8-2.3  |
| tetramethylthiuram disulphide | 0.5-0.7  |

\* \* \* \* \*